

(No Model.)

J. A. TOBIN.

COMPOUND STEEL ARMOR AND METHOD OF CONSTRUCTING THE SAME.

No. 351,297.

Patented Oct. 19, 1886.



Witnesses:

W. M. Davis  
Jack. L. Graham.

Inventor:

John A. Tobin

# UNITED STATES PATENT OFFICE.

JOHN A. TOBIN, OF WASHINGTON, DISTRICT OF COLUMBIA.

## COMPOUND STEEL ARMOR AND METHOD OF CONSTRUCTING THE SAME.

SPECIFICATION forming part of Letters Patent No. 351,297, dated October 19, 1886.

Application filed August 24, 1886. Serial No. 211,773. (No model.)

*To all whom it may concern:*

Be it known that I, JOHN A. TOBIN, a citizen of the United States, residing at Washington, in the District of Columbia, have invented 55  
5 a new and Improved Method in the Construction of Armor for Armor-Clad Ships.

What I claim as my invention is an improvement in the method of construction of compound steel armor for armor-clad ships, 10 floating batteries, and forts, of which the following is a full, clear, and exact description.

The nature of the improvement and the manner in which the same is carried into effect may be readily understood by reference to the 15 accompanying drawings.

Figure 1 represents a front and back plate of ship-side armor. Fig. 2 is a front and back plate of a turret. Fig. 3 is a cross-section showing deflective side armor attached to ship-side; Fig. 4, a quarter-section of a conning-tower, showing front and back plate; Fig. 5, a plan of a gun-shield, showing the front and back plate. Fig. 6 is a cross-section through Fig. 1, at  $f'g$ , showing cast bolt-holes  $k$  in 20  
25 back plate for fastening side armor, also ribs  $m$  on inside of plate  $b$  to keep it intact when subjected to the impact of projectiles.

Similar letters of reference designate corresponding parts throughout the different figures.

The front and back plates only are shown in Figs. 1, 2, 4, 5, and 6 to illustrate my mode of constructing armor.

In the operation of accomplishing my said 35 invention a pattern or templet one-quarter of the intended thickness of the armor is fashioned to suit the curvatures of the inside of the turret, conning-tower, or side of the ship requiring protection, and from a back plate is 40 cast in a green or dry sand mold lined with a refractory material, having sides and a bottom which form a part of the plate referred to. (See letter  $l$ , Figs. 1, 2, 3, 4, and 5 in the accompanying drawings.) The outside plate,  $b$ , is molded from a pattern or templet having a 45 thickness of about one-quarter of the finished plate, and may be so shaped as to suit any design of the exterior of any turret or armor-plate. The steel used in plate  $b$  contains certain toughening substances and carbon in sufficient quantity to insure a tensile strength of

about eighty tons per square inch. The cast-steel plates  $a$  and  $b$ , after being joined together by a simple contrivance, are heated in a heating-furnace until a white glowing heat is attained throughout the entire box or mold, the back and front plates of which compose the outside and inside of the armor. When the desired heat is obtained, the mold is withdrawn from the furnace and the cavity filled through 55 its open top with molten steel, (having carbon in sufficient quantity to insure a tensile strength of about forty tons per square inch,) which fuses with the hard-steel face and mild-steel back plate, uniting the whole into a compound solid and inseparable mass.

In Figs. 1 and 3,  $h$  represents wood backing behind armor. By my method of construction conning-towers may be made of solid inner and outer rings of any design and joined together 60  
65 in the manner described.

My improvement in the method of constructing compound steel armor for war-ships enables me to make with readiness, facility, and economy by casting, a large number of either 70 outside or inside turret or ship-side plates at the same time; also filling the cavities of several molds at one heat, thus rendering it, by this simple and economical process, unnecessary to occupy more than one furnace at any 75  
80 one time for the operation.

My deflective armor (see Fig. 3) having an inclined hard steel face to deflect and break up by impact the heaviest projectiles, a mild-steel back of great ductility (purified with 85 manganese and other methods) to hold intact the steel composing the intermediate layer and the hard-steel face, all of which, from its irregular and peculiar shape, cannot be otherwise accomplished without the employment 90 of a costly and extensive plant.

In my method of casting armor I may find it less expensive to make the plates  $b$ , Figs. 1, 2, and 3, of a hard and tough quality of cast-iron, or I may prefer to make the face and 95 back plates,  $a$  and  $b$ , both of a mild quality of steel and fill the cavity  $c$  with a hard tough quality of cast-iron or hard steel.

By my method of improvement in casting steel armor I may also find it economical and 100 advantageous to add layers of steel of varying degrees of hardness to armor already in use

by making a casting from a pattern which will represent the exterior of the turret or plate of the armor-clad, and after securing it heat the mass and fill the cavity with molten steel 5 in the manner already described and set forth.

I am aware that heretofore compound armor for war-ships and sea-coast defenses have been made by piling, rolling, and forging wrought-iron, which composes the back plate 10 of the present compound armor in use; also, that the thin hard-steel face composing the face of the armor is rolled from a hard-steel ingot, and that the space between them made by securing the two plates together is, after 15 being heated in a furnace, filled with molten steel and the mass finally subjected to the process of being rolled, hammered, and pressed into the desired shape by a costly and specially-adapted plant. I am also aware that 20 armor constructed of steel has been cast from ingots for war-ships and subjected to the process of being rolled and pressed into the desired shapes; also, that cast-steel blocks or 25 masses of uniform and varying degrees of hardness or temper have been broadly mentioned for ships' side armor, and I am also aware of the construction and method of manufacture of armor-plates, as shown in the Patent No. 239,155, and English patents of 30 Wilson, No. 4,746 of A. D. 1876, No. 3,472 of A. D. 1877; but I am not aware that my simple and expeditious method of constructing compound steel armor, as set forth and described, has ever been suggested or used by 35 any one.

Having fully described my improved method of constructing compound steel armor, and the mode of carrying out my invention, I would state that in the foregoing description of my 40 improved method of construction of cast-steel compound armor of varying degrees of hardness I have found it necessary, for the purpose of distinctness, to refer to certain well-known methods of operations as being adopted in the 45 course of construction of my improved com-

pound steel armor-plate, and therefore I do not claim as my invention any of said methods of operation, except when employed in the construction of my improved compound cast-steel armor-plate and ordnance in the manner 50 heretofore described and set forth.

What I do consider as both novel and original in my improvement is not only the simplified and expeditious manner of effecting the operation as described and set forth by me for 55 turrets, guns, gun-shields, conning-towers, and ships' side armor, but also the fact that by construction and arrangement of the compound steel plate purified by ferro-manganese and other methods I secure a sounder and more 60 reliable armor with a higher maximum of resistance to projectiles than can be secured by any other method of construction known to me. Finally, by my improved method of 65 making armor I avoid altogether the use of costly and extensive plants, made necessary by hammering, rolling, and pressing large plates to give them the desired form.

What I claim as my invention is—

1. A compound steel armor-plate composed 70 of a cast-steel back plate, of homogeneous mild steel molded to the proper form, with an inside-finished face of any particular shape, a hard face-plate of cast-steel molded and cast to any specific form, the two plates being connected and formed into a solid compound plate 75 by an intermediate layer of molten steel of medium tensile strength, substantially as set forth.

2. The process of making a compound cast- 80 steel armor-plate, which consists in casting separately to any desired form a back plate of homogeneous mild steel and a hard-steel face-plate and uniting the two plates with molten steel of medium tensile strength, as described. 85

JOHN A. TOBIN.

Witnesses:

GEO. W. ROUZER,  
WM. H. HARRIS.